

## UNITED STATES PATENT OFFICE

2,448,749

## TREATED PLANOGRAPHIC PRINTING PLATE

Charles H. Van Dusen, Jr., Willoughby, Ohio, assignor to Addressograph-Multigraph Corporation, Wilmington, Del., a corporation of Delaware

No Drawing. Application January 24, 1947,  
Serial No. 724,231

4 Claims. (Cl. 101—149.2)

**1** This invention relates to planographic printing. More particularly, this invention relates to paper planographic printing plates and to a process and solution for eliminating so-called finger prints and so-called resin specks or spots from the copies made from such paper planographic printing plates, including specks or spots caused by the naturally occurring wood rosin in the pulp from which such paper planographic printing plates are made.

As is well known in the art of planographic printing paper planographic printing plates, such as those which are composed of parchment and like cellulose materials, are particularly susceptible to picking up finger prints in handling and since such finger prints are formed from the fatty oil exudate of the skin they are receptive to the greasy or fatty acid containing inks employed in planographic printing and hence are reproduced on the copies during the planographic printing operation.

Moreover, so-called resin specks, including those formed from the natural rosins occurring in the wood used in making paper pulp, are frequently encountered in the copies made from paper planographic printing plates. These rosin specks are also receptive to the greasy or fatty acid-containing inks used in planographic printing and are reproduced as objectionable small black specks or spots in the copies formed during the planographic printing operation.

Various attempts have been made, and various materials have been used, heretofore to eliminate the reproduction of finger prints and rosin specks in the copies made from paper planographic printing plates. However, insofar as I am aware of all of such materials have either been unsuccessful in eliminating the reproduction of finger prints and so-called resin or rosin specks in the copies made from paper planographic printing plates or, if successful in so doing, have had the objectionable characteristic of weakening the image-reproducing characteristics of the image formed on the master paper planographic printing plate by means of the various planographic image-forming materials used for this purpose and which include typewriter ribbon image-forming materials, planographic image-forming inks, planographic image-forming crayons, and the like.

In and as the present invention I have, however, found a material which when applied as a water solution thereof to a dry or to a wet paper planographic printing plate, and the plate then dried, preparatory to placing a lithographic im-

age thereon, not only effectively eliminates or prevents the reproduction of any finger prints or resin or rosin particles or so-called resin or rosin specks in the copies made from the thus treated paper planographic printing plate but which likewise does not in any way weaken or otherwise interfere with the image-receptive or image-reproducing characteristics of the various planographic image-forming materials which may be employed in forming images on the treated paper planographic printing plates including typewriter image-forming materials, planographic image-forming inks, and the like.

Accordingly, an object of the present invention is to provide a novel process and solution for eliminating and preventing the reproduction of finger prints and so-called resin and rosin specks in the copies made from paper planographic printing plates.

Another object of the present invention is to provide a novel process and solution for eliminating and preventing the reproduction of finger prints in the copies made from paper planographic printing plates without in any way weakening or otherwise interfering with the image-receptive or image-reproducing characteristics of the various planographic image-forming materials which may be employed in forming images on such paper planographic printing plates including planographic image-forming typewriter ribbons, inks, crayons, and the like.

An additional object of the present invention is to provide a new and improved paper planographic printing plate impregnated or coated with the new solution of the present invention and which will not reproduce finger prints or resin or rosin specks in the copies reproduced therefrom but which, at the same time, does not in any way interfere with the image-receptive characteristics of or in any way interfere with or weaken the image-reproducing characteristics of the various image-forming materials which may be employed in forming images on paper planographic printing plates including planographic image-forming typewriter ribbons, inks, crayons, and the like.

In the practice of the present invention I prepare a five per cent solution, by weight, of 2 amino, 2 methyl, 1,3 propanediol (Commercial Solvents Corporation) in water and I then coat the printing surface of the paper planographic printing plate, which may be of a parchment or other cellulose base sheet, with this solution by brushing, spraying or otherwise applying the solution thereto. The thus treated plate is then

preferably run between a pair of squeeze rolls and allowed to dry whereupon it may be provided with a lithographic image by means of any suitable lithographic image-forming material, such as any of those hereinbefore referred to, and then treated with an aqueous planographic etching or dampening solution to condition the plate for use in a planographic printing operation. The resulting plate is thus a paper planographic printing plate impregnated with 2 amino, 2 methyl, 1,3 propanediol.

It has been found that parchment or like paper planographic printing plates treated with the new solution not only do not reproduce finger prints or resin or rosin specks in the copies made therefrom but have good image-receptive and good image-reproducing characteristics and that the new solution does not in any way weaken or otherwise interfere with the image-reproducing characteristics of the planographic image-forming material employed in forming the image thereon.

The effectiveness of the new process and solution were demonstrated by applying the new solution to approximately one-half of the surface area of the printing surface of a parchment planographic printing plate which was known to reproduce rosin specks due to the naturally occurring wood rosin therein. The other half of the printing surface of the said parchment plate was allowed to remain untreated. The thus treated parchment plate was then thoroughly dehydrated at room temperature and then finger printed throughout its entire printing surface including both the treated and the untreated areas thereof. One section of the thus treated parchment plate was thereupon exposed to natural diffused sunlight for a period of about four minutes and the other section was exposed to the rays of an ultra-violet lamp for a period of fifteen minutes. (Both of these treatments are known to exaggerate the image-reproducing characteristics of finger prints upon and of wood rosin specks in parchment or like paper planographic printing plates.) After having been thus exposed a lithographic image was applied to each section of the plate, by means of a suitable lithographic image-forming material, whereupon both sections of the thus treated and exposed parchment plate were treated with an aqueous planographic etching and repellent solution, fastened in position of use upon the plate cylinder of a rotary offset planographic duplicating press, and a satisfactory edition of copies run therefrom. However, the copies reproduced from those portions of the parchment planographic printing plate which was treated with the new solution did not exhibit either finger prints or so-called rosin specks whereas both finger prints and rosin specks appeared prominently in the copies reproduced from the untreated portions of the plate. Moreover, that area or section of the new plate which had been treated with the new solution exhibited equally as good image-reproducing characteristics and equally as long editions were reproduced therefrom as were exhibited by and reproduced from the other area or section of the plate which had not been so treated.

It has been found that the above named per-

centage, namely, five per cent, by weight, of 2 amino, 2 methyl, 1,3 propanediol in water is the optimum percentage when the new solution is applied to a dry paper planographic printing plate or mat. I have likewise found that when the new solution is applied to a wet paper planographic printing plate or mat the concentration of the solution and the quantity thereof applied is then preferably adjusted so that the resulting solution, thus diluted with and by the water in the wet paper planographic printing plate to which it is applied, is equivalent to a five (5) per cent solution, by weight, and when so controlled produces highly satisfactory solutions on paper planographic printing plates impregnated therewith. However, the exact amount of the material to be incorporated in a parchment or like paper planographic printing plate depends upon and may be adjusted to variable conditions including the condition of the sheet at the time the material is applied thereto, that is, whether wet or dry, its moisture content if nominally a so-called dry sheet, prevailing atmospheric or room humidity conditions, and the like.

It will thus be seen from the foregoing description that the present invention provides a novel process and solution for eliminating both finger prints and rosin specks in the copies reproduced from paper planographic printing plates treated with the new solution, and without interfering with either the image-receptive or the image-reproducing characteristics of paper planographic printing plates treated with the new solution, and thus provides a paper planographic printing plate having the desirable advantages and characteristics, and which accomplishes its intended objects, including those hereinbefore pointed out and others which are inherent in the invention.

I claim:

1. A paper planographic printing plate impregnated with 2 amino, 2 methyl, 1,3 propanediol.
2. A parchment planographic printing plate impregnated with 2 amino, 2 methyl, 1,3 propanediol.
3. A paper planographic printing plate impregnated with the dried residue of a five per cent water solution of 2 amino, 2 methyl, 1,3 propanediol.
4. A parchment planographic printing plate impregnated with the dried residue of a five per cent water solution of 2 amino, 2 methyl, 1,3 propanediol.

CHARLES H. VAN DUSEN, JR.

#### REFERENCES CITED

The following references are of record in the file of this patent:

#### UNITED STATES PATENTS

| Number    | Name    | Date          |
|-----------|---------|---------------|
| 2,373,287 | Bassist | Apr. 10, 1945 |

#### OTHER REFERENCES

Chemical Industries, vol. XLV, p. 666, The Nitroparaffins and their Derivations, December 7, 1939.